

Sept. 10, 1929.

C. L. BEAL

1,727,331

PROCESS OF COATING ALUMINUM ELECTROLYTICALLY

Filed Jan. 17, 1927

FIG - 1 -



FIG - 2 -



FIG - 3 -



INVENTOR,  
Carl L. Beal,  
BY *P. L. Stinchfield*  
ATTORNEY.

## UNITED STATES PATENT OFFICE.

CARL L. BEAL, OF ROCHESTER, NEW YORK, ASSIGNOR TO EASTMAN KODAK COMPANY, OF ROCHESTER, NEW YORK, A CORPORATION OF NEW YORK.

## PROCESS OF COATING ALUMINUM ELECTROLYTICALLY.

Application filed January 17, 1927. Serial No. 161,515.

This invention relates to processes of coating aluminum and alloys containing the same, electrolytically. One object of the invention is to provide a process in which an electrolytic coating of adequate density and adherence can be united to an aluminum surface in spite of the tendency of the latter to form a thin resistant film of oxide. Another object of the invention is to provide a process which will accomplish the above result at the minimum of trouble and expense. 10 Other objects will hereinafter appear.

In the accompanying drawing,—

Fig. 1 is a diagrammatic vertical section 15 on a reduced scale of one form of apparatus in which the first pretreatment step may be conveniently carried out;

Fig. 2 is a similar view of one form of apparatus in which the second pretreatment 20 step may conveniently be carried out;

Fig. 3 is a similar view of one form of apparatus in which the electrodeposition may conveniently take place.

It is well known that aluminum has been 25 difficult to coat reliably, because its surface, in contact with the air, rapidly forms a tenacious film, which even when it is thin, resists the adherence of an electrodeposited coating over it. For instance, it has been 30 difficult to produce a good reliable zinc coating electrolytically on aluminum.

I have found that this trouble can be avoided by first treating the surface of the aluminum in a dilute aqueous alkaline solution, 35 preferably hot, and then making it a cathode in an acid bath, these successive pretreatment steps bringing the surface to a condition in which it can be readily electroplated in a standard commercial bath, such as 40 an acid-sulfate zinc plating bath.

The first pretreatment step does not require any electrolysis, and is very rapid and economical. Various alkaline aqueous solutions may be employed, such as those of 45 sodium hydroxid, sodium carbonate, or trisodium phosphate. The concentration of the solution may vary considerably. I have found it convenient to work with one having a hydroxyl ion concentration of the same 50 order of magnitude as that of a 5% solu-

tion of trisodium phosphate. Working with such a solution at a temperature slightly below boiling, say 190 to 200° F. the surface to be treated requires only about a half minute immersion. Where it is undesirable 55 to carry any of this alkaline bath into the bath for the second pretreatment step, the article can be dipped for a few seconds in an acid bath, say 10% aqueous hydrochloric acid, but this is not indispensable, although 60 desirable.

The surface under treatment, after undergoing the action of the alkaline solution in the first step, is then made a cathode in an aqueous acid solution. For example, it may 65 be electrolyzed for about 3 to 5 minutes at a current density of 0.4 amperes per square inch with a voltage of around 2. The acid solution can be, for example, a 5% aqueous sulfuric acid one, but the concentration can 70 obviously be varied considerably, and any other acid can be substituted in an amount which will furnish a correspondingly sufficient hydrogen ion concentration.

It will be noted that the final cleaning, or 75 second pretreatment step takes place in an electrolyte which contains substantially no alkali metal salts. This is important because any considerable concentration of the ions of such metal causes conditions in the 80 cathode region, which favor further filming of the aluminum surface which forms the cathode. In my process the chief cations during the second pretreatment step are those of hydrogen ( $H^+$ ) and these tend to 85 dissolve the oxide and hydroxid that were previously formed or loosened during the first or alkaline pretreatment step. Moreover, the hydrogen polarization of the cathode surface prevents oxidation. While I do 90 not wish to be restricted to a particular theory of operation, since the above described pretreatment steps have been found in actual practice to be unexpectedly effective, nevertheless, I believe that hydrogen, in addition 95 to maintaining a non-oxidizing zone around the cathode, also mechanically eliminates some of the aluminum hydroxid coating, the bubbles acting on this coating, after the preliminary attack of the alkaline immersion. 100

The surface of the aluminum having undergone the pretreatment described above, can be plated in any well known acid-plating bath, such as the standard acid-sulfate 5 zinc plating bath operating at a current density of 0.1 to 0.2 upon the treated surface. As such baths are well known, the details of them are omitted here.

In the drawing, 1 represents any suitable 10 container in which is the dilute aqueous alkaline solution in which the article 3, having the surface of the readily oxidizable metal, is suspended in any suitable way, say by rod 4 and hook 5.

15 In Fig. 2 any suitable vessel 6 contains the dilute acid solution 7 in which the article to be treated 3 is immersed as the cathode, say by electroconducting hook 7 from cathode bar 8. Suitable anodes 9 are connected to anode bars 10. The bars 8 and 20 10 are connected to the poles of any suitable source of current 11. The anodes 9 are preferably of a material which does not foul the bath, such as carbon.

25 In Fig. 3 any suitable vessel 12 has suspended in the bath, as the cathode, the treated article 3 suspended by any suitable electroconducting hook 7 from cathode bar 8. The anodes 13 are connected to anode 30 bars 14. Bars 8 and 14 are connected to any suitable source of current 11. In the vessel is a standard electro-plating bath 15 of the type customarily used. In fact, Fig. 3 is merely a diagrammatic representation of 35 current electroplating practice.

Having thus described my invention, what I claim as new and desire to secure by Letters Patent is:

1. In the process of electroplating an aluminum surface, the steps of treating said surface in a dilute aqueous alkaline bath 40 without electrolysis, treating said surface as the cathode in an acid dilute aqueous bath under non-oxidizing conditions, and thereafter electrodepositing a coating upon said treated surface.

2. In the process of electroplating upon an aluminum surface, the steps of immersing said surface in an aqueous alkaline solution 50 to attack the film on said surface, treating said surface as the cathode in a dilute aqueous acid bath, substantially free from alkali metal ions to remove the attacked oxide coating and produce hydrogen polarization on said surface, and thereafter electroplating upon the thus prepared surface.

3. In the process of electrodepositing a coating upon an aluminum surface, the steps 60 of immersing said surface in a hot aqueous bath having an alkalinity of the order of magnitude of a 5% solution of trisodium phosphate, dipping the surface in a dilute aqueous acid solution, making said surface 65 a cathode in an aqueous acid bath, substan-

tially free from alkali metal ions, said bath having an acidity of the same order of magnitude as a 5% sulfuric acid bath, and thereafter electrodepositing upon the thus pretreated surface the desired coating.

Signed at Rochester, New York this 12th day of January 1927.

CARL L. BEAL.

70

75

80

85

90

95

100

105

110

115

120

125

130